

Sept. 30, 1924.

1,509,980

W. RAEBURN

CHAIR GLIDE AND METHOD OF MAKING THE SAME

Original Filed April 3, 1923

Fig 1



Fig 2



Fig 3



INVENTOR

Wm Raeburn  
BY  
Bartholomew  
ATTORNEYS

## UNITED STATES PATENT OFFICE.

WILLIAM RAEURN, OF WATERBURY, CONNECTICUT, ASSIGNOR TO THE MATTATUCK MANUFACTURING COMPANY, OF WATERBURY, CONNECTICUT, A CORPORATION OF CONNECTICUT.

## CHAIR GLIDE AND METHOD OF MAKING THE SAME.

Continuation of application Serial No. 629,574, filed April 3, 1923. This application filed November 24, 1923. Serial No. 676,676.

To all whom it may concern:

Be it known that I, WILLIAM RAEURN, a citizen of the United States, residing at Waterbury, county of New Haven, State of Connecticut, have invented certain new and useful Improvements in Chair Glides and Methods of Making the Same, of which the following is a full, clear, and exact description.

10 My invention relates to improvements in chair glides and methods of making the same and has for its object to provide a new and improved chair glide having a prong for securing the glide to the chair. It further has for its object to provide a chair glide having a hardened contact surface and a permanently secured tough prong which is soft relative to the contact surface though sufficiently hard for driving purposes.

15 This application is a continuation of my application Serial No. 629,574 filed April 3, 1923.

20 Heretofore chair glides have been made with integral prongs located at their peripheries and attempts have been made to produce satisfactory chair glides having central prongs. The chair glides with the central prongs have, however, heretofore been found to be unsatisfactory, for the reason 25 that either the contact surfaces were soft, or the prongs were so brittle as to be easily broken. By my invention a chair glide having a central prong is produced in which the contact surface is glass hard and in which 30 the prong, while of driving hardness, is softer than the contact surface, and so tough and tenacious as not to be liable to be broken either in driving or in use.

35 The following is a description of my invention and of a chair glide constructed and made in accordance therewith, reference being had to the accompanying drawings, in which,

40 Figure 1 is a bottom plan view of my improved chair glide;

45 Fig. 2 is a side elevation of the same; and

Fig. 3 is a partial section through the center of Fig. 1.

50 Referring more particularly to the drawings, 1 is a prong having a pointed end 2 and an enlargement 3, and 4 is a saucer-like

head secured to the prong 1 and providing the contact surface of the chair glide.

In the preferred form I make the prong and head of substantially the shapes shown. 55 The head is made of steel and when applied to the prong is in a soft condition so that it can be blanked out with gang tools in the ordinary manner and then secured to the prong by having swaged portions 5 60 forced over so as to embrace the enlargement thereof on an ordinary automatic nail machine such as is well known to those skilled in the art.

In embodying my invention in a structure having the mechanical features above described, I make the prong of some metal which is tough and highly resistant to heat and yet of driving hardness (by which I mean sufficiently hard so that a prong made 65 therefrom can be driven into the bottom of a chair leg made of wood such as ordinarily used for such legs, such for instance as oak, birch, hickory and the like), and which will not melt and will not become hard or brittle 70 so as to easily break when subjected to treatment such as is ordinarily employed for the hardening of steel. The metal which I prefer to use for securing these characteristics in a prong is Monel metal, a permanently 75 tough metal, whose composition is approximately 67 parts nickel, 30 parts copper with usually 2 or 3 parts of iron. Monel metal I describe as permanently tough since it does not become brittle when subjected to heat 80 treatment such as is used for hardening steel, and by the expression "permanently tough" I mean a metal having that characteristic.

The head of the glide is primarily made 90 of soft steel and is formed from blanks into the shape shown, and secured to the prong in the ordinary manner by an automatic nail machine such as is in common use for making headed nails of the general form shown. 95 This head is made of saucer-like form with its edge portion somewhat thinned and bent up sharply. Its edge proper is somewhat sharpened by the forming dies so as to bite into the wood of the leg and aid the prong 100 in resisting lateral thrust to which the glide may be subjected when in use.

After the prong and head have been assembled in the manner described I subject them to a heat treatment which will result in hardening the head and which will not materially affect the prong.

A suitable treatment for securing these results consists in dipping the assembled parts into a bath consisting of 75 per cent soda cyanide and 25 per cent soda ash heated to a temperature of about 1600°. The glides are placed in baskets and dipped into the bath being left therein for say, twenty minutes, or long enough to bring the glides to a temperature of 1500°. They are then removed and, when heated, plunged into water so as to be quickly cooled. This results in making the heads of the glides glass hard but does not harden the prong so as to make it brittle. After they are taken out they are placed in a rolling barrel and finished so as to give the contact surfaces of the heads a bright luster.

As will be evident to those skilled in the art, my invention permits of various modifications without departing from the spirit thereof or the scope of the appended claims.

What I claim is:

1. A chair glide consisting of a saucer-shaped hardened steel head and a softer tough prong of driving hardness, said head having swaged portions embracing one end of said prong so as to hold the two parts permanently together.

2. A chair glide consisting of a saucer-shaped hardened steel head and a softer tough prong of driving hardness, said head having swaged portions embracing one end of said prong so as to hold the two parts permanently together, said end having an enlargement embedded within the mass of said saucer-shaped head.

3. A chair glide consisting of a saucer-shaped steel head of glass hardness and a softer tough prong of driving hardness, said

head having swaged portions embracing one end of said prong so as to hold the two parts permanently together, said saucer-shaped head having a sharpened edge adapted to aid the prong in resisting sidewise thrust.

4. A chair glide comprising a saucer-shaped head of hardened steel and a prong of Monel metal having one end embraced by swaged portions of said saucer-shaped head so as to hold the two parts permanently together.

5. A chair glide comprising a saucer-shaped head of glass hard steel and a prong of Monel metal having one end embraced by swaged portions of said saucer-shaped head so as to hold the two parts permanently together.

6. The method of making chair glides and similar articles, which consists in forming a permanently tough heat-resisting metallic prong of driving hardness, swaging portions of a soft steel head about the end of the prong so as to permanently secure the head thereto, and subjecting the parts thus assembled to a hardening heat treatment so as to harden the steel head.

7. The method of making chair glides and similar articles, which consists in forming a prong of Monel metal, swaging portions of a soft steel head about the end of the prong so as to permanently secure the head thereto, and subjecting the parts thus assembled to a hardening heat treatment so as to harden the steel head.

8. The method of making chair glides and similar articles, which consists in forming a permanently tough heat-resisting metallic prong of driving hardness, swaging portions of a soft steel head about the end of the prong so as to permanently secure the head thereto, subjecting the parts thus assembled to a heated cyanide bath and quickly cooling the same when in a heated condition.

WILLIAM RAEURN.